

# UNITED STATES PATENT OFFICE.

ANTON LEDERER, OF ATZGERSDORF, NEAR VIENNA, AUSTRIA-HUNGARY.

MANUFACTURE OF EXCEEDINGLY-THIN METALLIC GLOWING FILAMENTS FOR ELECTRIC INCANDESCENT LAMPS.

1,035,883.

Specification of Letters Patent. Patented Aug. 20, 1912.

No Drawing.

Application filed April 3, 1906. Serial No. 309,716.

To all whom it may concern:

Be it known that I, ANTON LEDERER, a subject of the Empire of Austria-Hungary, residing at No. 83 Atzgersdorf, near Vienna, 5 in the Province of Lower Austria and Empire of Austria-Hungary, have invented new and useful Improvements in the Manufacture of Exceedingly-Thin Metallic Glowing Filaments for Electric Incandescent Lamps, 10 of which the following is a specification.

My invention relates to improvements in the manufacture of metallic glowing filaments for electric incandescent lamps and has for its object the production of exceedingly thin filaments from comparatively thick raw filaments, obtained by forcing the material under treatment through a die of a comparatively large diameter.

With economical burning electric incandescent lamps having metallic glowing filaments and being designated for higher tensions and less illuminating power as for example for 110 volts and 10 candles' power, the diameter of the filament need not be 25 greater than some thousandths of a millimeter.

Most of the metallic glowing filaments are produced by forcing pastes through suitable dies; now it is very difficult from the technical point of view to make dies having a diameter of about 0.005 to 0.008 of a millimeter and consequently the manufacture of metallic glowing filaments of such small diameters is nearly impossible.

35 The process according to this invention allows of the manufacture of filaments even of the small diameters as above indicated and of all metals and metal alloys; I will describe the same as applied to the manufacture of filaments of tungsten or of molybdenum.

45 Finely powdered metallic tungsten is intimately mixed with also finely powdered oxid of zinc or with sulfid of zinc and with an organic agglutinant in such a quantity that the finished filament does not contain any carbon. From this mixture a paste is made by grinding. The paste is then forced through a die in order to obtain filaments 50 which are heated under exclusion of air. Care is to be taken that temperature be not raised too high because in this case the added substance might easily be volatilized. The filaments thus obtained are glowed in 55 an inert atmosphere or *in vacuo* by the

electric current passed therethrough, whereby the oxid of zinc or the sulfid of zinc combines with the carbon of the agglutinant and is volatilized partly as carbonic oxide or as carbonic acid and partly as sulfuret of carbon and as a metallic zinc. The filament which originally was of a greater volume visibly shrinks and sinters. 60

I found that raw filaments of a diameter of 0.1 mm. before treatment have shown a 65 diameter of only 0.01 mm. after having been submitted to the process above described.

It is obvious, that not only the oxid of zinc but also the oxid of cadmium and other easily reducible oxides or sulfids of other 70 volatile metals may be used in this process.

Reduction takes place about according to the formula below:



Of course, this reaction may be reversed, that is to say: A metallic oxid or sulfid may be mixed with metallic zinc and with an organic agglutinant and the mixture be 80 worked into filaments, the result will be the same and reaction take place as indicated by the formula:



A further modification of the process consists in preparing filaments of a paste composed of a metallic oxid and of oxid of zinc or of cadmium or of a sulfid of a metal; the 90 following equations show the process:



The quantities of the added substance may 95 be varied within the largest limits without influencing with in any way the quality of the final product.

It is obvious that filaments of alloys of several other refractory metals may be 100 manufactured in the same way.

What I claim as my invention, and desire to secure by Letters Patent, is:—

1. The process of manufacturing exceedingly thin filaments of refractory metal for 105 electric incandescent lamps, which consists in forming a paste composed of the metal in a finely divided condition and an easily reducible and readily volatilizable metallic compound and a suitable agglutinant, form- 110

ing relatively large filaments from the paste thus obtained and glowing these filaments in the absence of oxygen other than that contained in the paste by an electric current, thereby volatilizing the added substances and reducing the thickness of the filaments and leaving pure metallic filament of the required cross section.

2. The process of manufacturing exceedingly thin filaments of refractory metal for electric incandescent lamps, consisting in forming a paste containing the metal and oxid of zinc and a suitable agglutinant, forming filaments of this paste by pressure and glowing the filaments in the absence of oxygen other than that contained in the paste by means of an electric current, thereby sintering the filaments and volatilizing

the content of the paste except the metal designed to form the filament.

3. The process of forming filaments for incandescent electric lamps, which consists in heating in an inert atmosphere a mixture of tungsten, a readily volatilizable metal and carbon in the presence of sufficient oxygen combined in the paste to oxidize all the carbon, and by such heating oxidizing the carbon, driving off the resultant gas and volatilizing the volatilizable metal.

In testimony whereof I have signed my name to this specification in the presence of two subscribing witnesses.

ANTON LEDERER.

Witnesses:

JOHANN LUX,  
ALVESTO S. HOGUE.